# EUROPEAN PATENT SPECIFICATION

(11) **EP 3 889 305 B1**
(45) Date of publication and mention of the grant of the patent: **10.04.2024**
(21) Application number: 19889727.4
(22) Date of filing: 29.11.2019
(51) Int. Cl.: C22C 38/58, C22C 38/50, C22C 38/48, C22C 38/44, C22C 38/04, C22C 38/02, C22C 38/06, C22C 38/00, C21D 8/02

(54) **HIGH-STRENGTH STEEL PLATE HAVING EXCELLENT LOW-TEMPERATURE FRACTURE TOUGHNESS AND ELONGATION RATIO, AND MANUFACTURING METHOD THEREFOR**
HOCHFESTE STAHLPLATTE MIT AUSGEZEICHNETER TIEFTEMPERATURBRUCHZÄHIGKEIT UND STRECKVERHÄLTNIS UND HERSTELLUNGSVERFAHREN DAFÜR
PLAQUE D'ACIER À HAUTE RÉSISTANCE AYANT UN EXCELLENT RAPPORT DE TÉNACITÉ À LA RUPTURE ET D'ALLONGEMENT À BASSE TEMPÉRATURE ET PROCÉDÉ DE FABRICATION ASSOCIÉ

(30) Priority: 30.11.2018 KR 20180151565
(43) Date of publication of application: 06.10.2021
(73) Proprietor: POSCO Co., Ltd, Pohang-si, Gyeongsangbuk-do 37859 (KR)
(72) Inventor: YOO, Jang-Yong, Pohang-si, Gyeongsangbuk-do 37877 (KR); BAE, Moo-Jong, Pohang-si, Gyeongsangbuk-do 37877 (KR); PARK, Yoen-Jung, Pohang-si, Gyeongsangbuk-do 37877 (KR)
(74) Representative: Meissner Bolte Partnerschaft mbB
(86) International application number: PCT/KR2019/016785
(87) International publication number: WO 2020/111891

(56) References cited:
- WO-A1-2009/072753
- JP-A- 2015 199 987
- KR-A- 20090 058 058
- KR-A- 20120 073 408
- KR-A- 20130 073 472
- KR-A- 20130 073 472
- KR-A- 20140 083 540
- KR-A- 20140 083 540
- KR-B1- 101 889 182

## Description

### [Technical Field]

The present invention relates to a high-strength steel plate and a manufacturing method therefor., and more particularly, to a high-strength steel plate for a pipeline capable of being stably used even in a harsh environment by having high strength characteristics through optimization of a steel composition, a microstructure, and a manufacturing process and having excellent low-temperature fracture toughness and elongation ratio, and a manufacturing method therefor.

### [Background Art]

Recently, as oilfield development has been carried out in cold regions such as Siberia and Alaska where climatic conditions are poor, projects to transport abundant gas resources from oil-rich regions to consumption regions through pipelines have been actively conducted. A steel used in such a pipeline project should necessarily have durability against deformation of the pipeline due to a cryogenic temperature and frost heave (a phenomenon of pushing up the surface of Earth when the ground freezes at the change of seasons) as well as a pressure of a transport gas, and is thus required to have high strength characteristics and excellent drop weight tearing test (DWTT) fracture toughness, and high elongation ratio characteristics.

A DWTT percent ductile fracture is a kind of index for determining whether or not a steel for a pipeline has brittle fracture arrestability for being safely used at a low temperature. In general, the pipelines provided in the cold regions are required to have a DWTT percent shear of 85% or more at -20°C in a pipe state. In order to secure the DWTT percent shear of 85% or more at -20°C in a pipe state, a DWTT percent shear of a steel plate provided for manufacturing a pipe should satisfy 85% or more at -30°C.

In general, it has been known that DWTT property has a deep association with an effective grain size of the steel plate. The effective grain size is defined as a size of grains having a high angle grain boundary, and as the effective grain size is refined, crack arrestability increases. The reason therefor that a propagation path of a crack changes at an effective grain boundary when the crack is initiated and propagated.

In order to refine the effective grain size, a method of performing accelerated cooling immediately after rolling is widely used. A mixed structure of acicular ferrite and bainite may be implemented by accelerated cooling immediately after rolling. However, a microstructure formed through usual accelerated cooling has high hardness because carbon (C) is supersaturated in grains, and accordingly, exhibits inferior ductility such as a uniform elongation ratio less than 9% and a total elongation ratio less than 20%. As a result, formability at the time of forming a pipe is lowered, and local stress concentration is easily generated at the time of applying external deformation, and thus, stability of the pipe is significantly reduced.

Therefore, in the manufacture of a steel plate for a pipeline, a manufacturing method for a steel plate for a pipeline having excellent low-temperature fracture toughness and having excellent ductility by having a uniform elongation ratio of 9% or more and a total elongation ratio of 28% or more by suppressing deterioration of an elongation ratio of the steel plate manufactured by accelerated cooling has been demanded.

In the related art, there were studies on a steel plate having an excellent elongation ratio and low-temperature fracture toughness. In this regard, Patent Literature 1 proposes a method of manufacturing a steel containing a mixed structure of 30 of 60% of equiaxed ferrite and 40 to 70% of bainite in terms of area fraction as a microstructure by non-recrystallized-region-rolling a steel containing nickel (Ni), niobium (Nb), and molybdenum (Mo) at a rolling reduction of 65% or more, primarily cooling the steel to a Bs temperature at a cooling rate of 15 to 30°C/s, and secondarily cooling the steel to a temperature range of 350 to 500°C at a cooling rate of 30 to 60°C/s.

However, in Patent Document 1 in which low-temperature rolling is performed on a steel plate having a thickness of 20 mm or more, there is a technical difficulty in applying the corresponding process condition to a steel plate having a thickness less than 20 mm. The reason is that the steel plate having the thickness less than 20 mm is subjected to low-temperature rolling and then cooled rapidly, and it is thus difficult to secure desired low-temperature fracture toughness, strength, and elongation ratio in an entire length direction of the steel plate, particularly, at a rear end portion of the steel plate.

Patent Document 2 teaches a steel plate for a line pipe having superior uniform elongation ratio and low-temperature fracture toughness and a manufacturing method of the steel plate which comprises by weight%, 0.04-0.10% carbon, 0.05-0.50% silicon, 1.4-2.0% manganese, 0.01-0.05% aluminum, 0.005-0.02% titanium, 0.002-0.01% nitride, 0.02-0.07% niobium, 0.05-0.3% chromium, 0.1-0.4% nickel, 0.05-0.3% molybdenum, identical to or less than 0.015% phosphorus, equal to or less than 0.005% sulfate, 0.0005-0.004% calcium, and a balance of iron and unavoidable impurities, of which a microstructure comprises on area percentage, 50-65% ferrite, 30-40% bainite, 5-10% martensite-austenite constituent, in which the average valid particle size of the ferrite is identical to or less than 10pm, and the average valid particle size of the bainite is identical to or less than 20um.

### (Related Art Document)

(Patent Document 1) KR 10 2013 0 073 472 A
(Patent Document 2) KR 10 2014 0 083 540 A

### [Disclosure]

### [Technical Problem]

An aspect of the present invention is to provide a high-strength steel plate having excellent low-temperature toughness, and a manufacturing method therefor.

### [Technical Solution]

According to an aspect of the present invention, a high-strength steel plate having excellent low-temperature fracture toughness and elongation ratio contains: by wt%, 0.05 to 0.1% of carbon (C), 0.05 to 0.5% of silicon (Si), 1.4 to 2.0% of manganese (Mn), 0.01 to 0.05% of aluminum (Al), 0.005 to 0.02% of titanium (Ti), 0.002 to 0.01% of nitrogen (N), 0.04 to 0.07% of niobium (Nb), 0.05 to 0.3% of chromium (Cr), 0.05 to 0.4% of nickel (Ni), 0.02% or less of phosphorus (P), 0.005% or less of sulfur (S), 0.0005 to 0.004% of calcium (Ca), remaining iron (Fe), and inevitable impurities; and 20 to 60 area% of ferrite, 35 to 75 area% of bainite and 5 area% or less of martensite-austenite constituent as a microstructure, wherein a grain size of upper 80% of high angle grain sizes based on 15° in a central portion of the high-strength steel plate is 70 µm or less, wherein the steel plate optionally further comprises 0.3 wt% or less of molybdenum (Mo), wherein a thickness of the high-strength steel plate is less than 20 mm, wherein a yield strength of the high-strength steel plate is 485 MPa or more, wherein a total elongation ratio of the high-strength steel plate is 28% or more, wherein a uniform elongation ratio of the high-strength steel plate with respect to a rolling orthogonal direction is 9% or more, and wherein a drop weight tearing test (DWTT) percent ductile shear of the high-strength steel plate at -30°C with respect to a rolling orthogonal direction of the steel plate is 85% or more wherein the yield strength and the elongation ratio were evaluated by performing a room temperature tensile test with respect to a rolling orthogonal direction.

According to another aspect of the present invention, a manufacturing method for a high-strength steel plate having excellent low-temperature fracture toughness and elongation ratio includes: reheating a slab containing, by wt%, 0.05 to 0.1% of carbon (C), 0.05 to 0.5% of silicon (Si), 1.4 to 2.0% of manganese (Mn), 0.01 to 0.05% of aluminum (Al), 0.005 to 0.02% of titanium (Ti), 0.002 to 0.01% of nitrogen (N), 0.04 to 0.07% of niobium (Nb), 0.05 to 0.3% of chromium (Cr), 0.05 to 0.4% of nickel (Ni), 0.02% or less of phosphorus (P), 0.005% or less of sulfur (S), 0.0005 to 0.004% of calcium (Ca), remaining iron (Fe), and inevitable impurities; maintaining and extracting the slab; recrystallized-region-rolling the maintained and extracted slab in a temperature range of Tnr or higher; non-recrystallized-region-rolling the recrystallized-region-rolled material at a total reduction ratio of 30% or more; and cooling the non-recrystallized-region-rolled steel plate to a temperature range of (Bs - 80°C) to Bs, wherein the non-recrystallized-region-roll starts in a temperature range of Tnr or lower and ends in a temperature range of (Ar3 + 100°C) or higher, wherein the slab plate optionally further comprises 0.3 wt% or less of molybdenum (Mo), wherein a reheating temperature range of the slab is 1140 to 1200°C, wherein a maintaining and extracting temperature range of the slab is 1140 to 1200°C, wherein the non-recrystallized-region-rolled steel plate is cooled at a cooling rate of 10 to 50°C/s, wherein the cooling of the non-recrystallized-region-rolled steel plate starts in the temperature range of (Ar3 + 30°C) or higher, and wherein the Tnr, Ar3 and Bs is calculated by Equations 1 to 3 below. $\begin{matrix}Tnr \left(°C\right) = 887 + 464 * \left[C\right] + 6445 * \left[Nb\right] - \\ 644 * {\left[Nb\right]}^{\left(1/2\right)} + 732 * \left[V\right] - 230 * {\left[V\right]}^{\left(1/2\right)} + 890 * \left[Ti\right] + 363 * \left[Al\right] - \\ 357 * \left[Si\right]\end{matrix}$ $\begin{matrix}Ar3 \left(°C\right) = 910 - 273 * \left[C\right] - 74 * \left[Mn\right] - 57 * \left[Ni\right] \\ - 16 * \left[Cr\right] - 9 * \left[Mo\right] - 5 \left[Cu\right]\end{matrix}$ $\begin{matrix}Bs \left(°C\right) = 830 - 270 * \left[C\right] - 90 * \left[Mn\right] - 37 * \left[Ni\right] \\ - 70 * \left[Cr\right] - 83 * \left[Mo\right]\end{matrix}$
where, [C], [Si], [Mn], [Al], [Ti], [Nb], [V], [Cr], [Mo], and [Cu] refer to wt% of respective alloy compositions, and when a corresponding alloy composition is not contained, calculation is performed by replacing a value of the corresponding alloy composition with 0.

The technical solution does not enumerate all of the features of the present invention, and various features of the present invention and advantages and effects according to the various features will be understood in more detail with reference to the following specific exemplary embodiments.

### [Advantageous Effects]

As set forth above, according to an exemplary embodiment in the present invention, a steel plate particularly suitable as a material for a pipeline by having high strength characteristics and having excellent low-temperature fracture toughness and elongation ratio, and a manufacturing method therefor is provided.

### [Description of Drawings]

FIG. 1 is a photograph of Specimen 2 of Inventive Example observed with an optical microscope.
FIG. 2 is graphs illustrating results obtained by measuring high angle grain boundary grain sizes based on 15° of Specimen 2 using electron backscatter diffraction (EBSD).
FIG. 3 is a photograph of Specimen 18 of Inventive Example observed with an optical microscope.
FIG. 4 is graphs illustrating results obtained by measuring high angle grain boundary grain sizes based 15° of Specimen 18 using an EBSD.

### [Best Mode for Invention]

The present invention relates to a high-strength steel plate having excellent low-temperature fracture toughness and elongation ratio, and a manufacturing method therefor, and exemplary embodiments in the present invention will hereinafter be described. Exemplary embodiments in the present invention may be modified to have several forms, and it is not to be interpreted that the scope of the present invention is limited to exemplary embodiments described below. The present exemplary embodiments are provided in order to further describe the present invention in detail to those skilled in the art to which the present invention pertains.

Hereinafter, compositions of a steel according to the present invention will be described in more detail. Hereinafter, unless otherwise indicated, % indicating a content of each element is based on weight.

A high-strength steel plate having excellent low-temperature fracture toughness and elongation ratio according to an exemplary embodiment in the present invention contains: by wt%, 0.05 to 0.1% of carbon (C), 0.05 to 0.5% of silicon (Si), 1.4 to 2.0% of manganese (Mn), 0.01 to 0.05% of aluminum (Al), 0.005 to 0.02% of titanium (Ti), 0.002 to 0.01% of nitrogen (N), 0.04 to 0.07% of niobium (Nb), 0.05 to 0.3% of chromium (Cr), 0.05 to 0.4% of nickel (Ni), 0.02% or less of phosphorus (P), 0.005% or less of sulfur (S), 0.0005 to 0.004% of calcium (Ca), remaining iron (Fe), and inevitable impurities.

In addition, the high-strength steel plate having excellent low-temperature fracture toughness and elongation ratio according to an exemplary embodiment in the present invention may further contain, by wt%, 0.3% or less of molybdenum (Mo).

### Carbon (C): 0.05 to 0.1%

Carbon (C) is an element that is the most effective in improving strength of a steel. In addition, when an amount of added carbon (C) is less than a predetermined level, expensive alloying elements such as molybdenum (Mo) and nickel (Ni) need to be added in a large amount in order to secure the strength of the steel, which is not preferable in terms of economy. In the present invention, a lower limit of a content of carbon (C) is limited to 0.05% in order to achieve such an effect. However, when carbon (C) is added in an excessive amount, it is not preferable in terms of weldability, formability, toughness, and the like of the steel. Thus, in the present invention, an upper limit of the content of carbon (C) is limited to 0.1%. Therefore, the content of carbon (C) of the present invention is in the range of 0.05 to 0.1%, and may be more preferably in the range of 0.05 to 0.095%.

### Silicon (Si): 0.05 to 0.5%

Silicon (Si) is an element useful for deoxidation of a molten steel, and is also an element that contributes to improving strength of the steel by solid solution strengthening. In the present invention, a lower limit of a content of silicon (Si) is limited to 0.05% in order to achieve such an effect. A more preferable lower limit of the content of silicon (Si) may be 0.1%. However, since silicon (Si) is an element having strong oxidation properties, it is preferable to limit an upper limit of the content of silicon (Si) to a predetermined range. That is, when silicon (Si) is added in an excessive amount, it causes red scale formation at the time of hot rolling, which is not preferable in terms of surface quality, and has an undesirable influence on toughness of a weld zone. Thus, in the present invention, the upper limit of the content of silicon (Si) is limited to 0.5%. A more preferable upper limit of the content of silicon (Si) may be 0.4%.

### Manganese (Mn): 1.4 to 2.0%

Manganese (Mn) is an element that is effective in solid solution strengthening of the steel. In the present invention, a lower limit of a content of manganese (Mn) is limited to 1.4% in order to secure high strength properties of the steel. However, when manganese (Mn) is added in an excessive amount, a segregation portion may be formed over a wide range in a central portion of a thickness at the time of casting a slab in a steelmaking process, which is not preferable in terms of weldability of a final product. Thus, in the present invention, an upper limit of the content of manganese (Mn) is limited to 2.0%. A more preferable upper limit of the content of manganese (Mn) may be 1.8%.

### Aluminum (Al): 0.01 to 0.05%

Aluminum (Al) is a representative element that is added as a deoxidizing agent along with silicon (Si). In addition, aluminum (Al) is an element that contributes to improving strength of the steel by solid solution strengthening. In the present invention, a lower limit of a content of aluminum (Al) is limited to 0.01% in order to achieve such an effect. A more preferable lower limit of the content of aluminum (Al) may be 0.015%. However, when aluminum (Al) is excessively added, it is not preferable in terms of impact toughness. Thus, in the present invention, an upper limit of the content of aluminum (Al) is limited to 0.05%. A more preferable upper limit of the content of aluminum (Al) may be 0.04%.

### Titanium (Ti): 0.005 to 0.02%

Titanium (Ti) is an element that forms TiN precipitates in a solidification process of the steel to suppress growth of austenite grains in a slab heating and hot rolling process, and thus refines a grain size of a final structure. In the present invention, a lower limit of the content of titanium (Ti) is limited to 0.005% in order to achieve a toughness improvement effect of the steel according to the refinement of the final structure. A more preferable content of titanium (Ti) may be 0.008%. However, when titanium (Ti) is excessively added, TiN is coarsely precipitated at the time of heating the slab, which is not suitable for the refinement of the final structure. Thus, in the present invention, an upper limit of the content of titanium (Ti) is limited to 0.02%. A more preferable upper limit of the content of titanium (Ti) may be 0.018%.

### Nitrogen (N): 0.002 to 0.01%

Nitrogen (N) is solid-dissolved in the steel and then precipitated to serve to increase strength of the steel, and it is known that such a strength improvement effect is much greater than that of carbon (C). In addition, in the present invention, TiN is formed through a reaction between titanium (Ti) and nitrogen (N) and it is intended to suppress growth of grains in a reheating process. Thus, a lower limit of a content of nitrogen (N) is limited to 0.002%. However, when nitrogen (N) is excessively added, nitrogen (N) exists in a form of solid solution nitrogen (N) rather than a form of TiN precipitates, so that toughness of the steel may be significantly reduced. Thus, in the present invention, an upper limit of the content of nitrogen (N) is limited to 0.01%. A preferable upper limit of the content of nitrogen (N) may be 0.006 %, and a more preferable upper limit of the content of nitrogen (N) may be 0.005%.

### Niobium (Nb): 0.04 to 0.07%

Niobium (Nb) is an element that is very useful for refining grains, and is an element that significantly contributes to improving strength of the steel by promoting formation of acicular ferrite or bainite, which is a high-strength structure. In addition, since high-temperature rolling is inevitable for a steel plate having a thickness less than 20 mm, which is a target thickness in the present invention, niobium (Nb) that has the greatest effect on an increase in a non-recrystallization temperature needs to be added in a predetermined amount or more. Thus, in the present invention, a lower limit of a content of niobium (Nb) is limited to 0.04%. However, when niobium (Nb) is excessively added, weldability of the steel may be deteriorated. Thus, in the present invention, an upper limit of the content of niobium (Nb) is limited to 0.07%. A preferable upper limit of the content of niobium (Nb) may be 0.06%.

### Chromium (Cr): 0.05 to 0.3%

Chromium (Cr) is an element that improves hardenability and is an element that is effective in increasing strength of the steel. In addition, chromium (Cr) is an element that contributes to improving a uniform elongation ratio by promoting formation of martensite-austenite constituent (MA) at the time of accelerated cooling. In the present invention, a lower limit of a content of chromium (Cr) is limited to 0.05% in order to achieve such an effect. A more preferable lower limit of the content of chromium (Cr) may be 0.08%. However, when chromium (Cr) is excessively added, deterioration of weldability of the steel may be caused. Thus, in the present invention, an upper limit of the content of chromium (Cr) is limited to 0.3%. A preferable upper limit of the content of chromium (Cr) may be 0.25%, and a more preferable upper limit of the content of chromium (Cr) may be 0.2%.

### Nickel (Ni): 0.05 to 0.4%

Nickel (Ni) is an element that effectively contributes to improving toughness and strength of the steel. In the present invention, a lower limit of a content of nickel (Ni) is limited to 0.05% in order to achieve such an effect. However, nickel (Ni) is an expensive element, and excessive addition of nickel (Ni) is not preferable in terms of economy Thus, in the present invention, an upper limit of a content of nickel (Ni) is limited to 0.4%. A preferable upper limit of the content of nickel (Ni) may be 0.3%, and a more preferable upper limit of the content of nickel (Ni) may be 0.25%.

### Phosphorus (P): 0.02% or less

Phosphorus (P) is a representative impurity element that exists in the steel, and is mainly segregated in a central portion of the steel plate to cause a decrease in toughness of the steel, and it is thus preferable to manage phosphorus (P) at a level as low as possible. However, in order to completely remove phosphorus (P) in the steel, an excessive cost and time are required in the steelmaking process, which is not preferable in terms of economy. Thus, in the present invention, a content of phosphorus (P) is limited to 0.02% or less. A more preferable content of phosphorus (P) may be 0.015% or less.

### Sulfur (S): 0.005% or less

Sulfur (S) is also a representative impurity element that exists in the steel, and is an element that combines with manganese (Mn) or the like in the steel to form nonmetallic inclusions such as MnS, and accordingly, significantly impairs toughness and strength of the steel. Thus, it is preferable to manage sulfur (S) at a level as low as possible. However, in order to completely remove sulfur (S) in the steel, an excessive cost and time are required in the steelmaking process, which is not preferable in terms of economy. Thus, in the present invention, a content of sulfur (S) is limited to 0.005% or less. A more preferable content of sulfur (S) may be 0.003% or less.

### Calcium (Ca): 0.0005 to 0.004%

Calcium (Ca) is an element that is effective in suppressing crack formation around nonmetallic inclusions by spheroidizing nonmetallic inclusions such as MnS. In the present invention, a lower limit of a content of calcium (Ca) is limited to 0.0005% in order to achieve such an effect. However, when calcium (Ca) is excessively added, a large amount of CaO-based inclusions is formed to cause a decrease in impact toughness. Thus, in the present invention, an upper limit of a content of calcium (Ca) is limited to 0.004%. A preferable upper limit of the content of calcium (Ca) may be 0.002%.

### Molybdenum (Mo): 0.3% or less

Molybdenum (Mo) is an element that is effective in securing both of high strength and high toughness by promoting formation of bainite, which is a low-temperature transformation structure. Therefore, in the present invention, molybdenum (Mo) may be selectively added in order to achieve such an effect. However, molybdenum (Mo) is an expensive element and it is not preferable in terms of economy to add molybdenum (Mo) in an excessive amount. Thus, in the present invention, an upper limit of a content of molybdenum (Mo) may be limited to 0.3%.

In the present invention, in addition to the steel compositions described above, the remainder contains Fe and inevitable impurities. The inevitable impurities may be unintentionally mixed in a general steelmaking process and may not be completely excluded, and those skilled in a general steelmaking field may easily understand the meaning of the inevitable impurities. In addition, the present invention does not entirely exclude addition of a composition other than the steel compositions described above.

A microstructure according to the present invention will hereinafter be described in more detail.

The steel plate according to an exemplary embodiment in the present invention contains ferrite and bainite as a microstructure, and further contain martensite-austenite constituent. Fractions of the ferrite and the bainite is 20 to 60 area% and 35 to 75 area%, respectively, and a fraction of the martensite-austenite constituent is 5 area% or less.

The steel plate according to the present invention contains ferrite having a fine high angle grain boundary in an area of 20% or more, and may thus effectively secure low-temperature drop weight tearing test (DWTT) characteristics. In addition, the steel plate according to the present invention contains the ferrite in an area of 60% or less and contains the bainite in an area of 35% or more, and thus secure a yield strength of 485 MPa or more. However, in the present invention, a fraction of the bainite is limited to 75 area% or less in order to prevent the high angle grain boundary from becoming excessively coarse, and accordingly, low-temperature DWTT characteristics may be effectively secured. In addition, the martensite-austenite constituent has an undesirable influence on the low-temperature DWTT characteristics, and it is thus preferable to suppress a fraction of the martensite-austenite constituent as much as possible. Therefore, in the present invention, the fraction of the martensite-austenite constituent is limited to 5 area% or less.

In addition, the steel plate according to an exemplary embodiment in the present invention has a grain size of 70 um or less in upper 80% of high angle grain sizes based on 15° in a central portion of the steel plate. That is, in the present invention, effective grain sizes may be refined by refining the high angle grain sizes, and accordingly, low-temperature DWTT characteristics may be effectively secured. Here, the central portion of the steel plate may be interpreted as an area including a point of t/2, and may also be interpreted as an area of a point of t/4 to 3*t/4 (t: thickness (mm) of steel plate).

The steel plate according to an exemplary embodiment in the present inventionhas a thickness less than 20 mm, and a preferable thickness of the steel plate may be 16 mm or less. In addition, the steel plate according to an exemplary embodiment in the present invention has a yield strength of 485 MPa or more, a total elongation ratio of 28% or more, and a uniform elongation ratio of 9% or more with respect to a rolling orthogonal direction, and has a DWTT percent ductile fracture of 85% or more at -30°C with respect to the rolling orthogonal direction of the steel plate. Therefore, in the present invention, a steel plate particularly suitable as a material for a pipeline by effectively securing strength, low-temperature fracture toughness, and an elongation ratio in spite of having the thickness less than 20 mm may be provided.

A manufacturing method according to the present invention will hereinafter be described in more detail.

The high-strength steel plate having excellent low-temperature fracture toughness and elongation ratio according to an exemplary embodiment in the present invention is manufactured by reheating a slab containing, by wt%, 0.05 to 0.1% of carbon (C), 0.05 to 0.5% of silicon (Si), 1.4 to 2.0% of manganese (Mn), 0.01 to 0.05% of aluminum (Al), 0.005 to 0.02% of titanium (Ti), 0.002 to 0.01% of nitrogen (N), 0.04 to 0.07% of niobium (Nb), 0.05 to 0.3% of chromium (Cr), 0.05 to 0.4% of nickel (Ni), 0.02% or less of phosphorus (P), 0.005% or less of sulfur (S), 0.0005 to 0.004% of calcium (Ca), remaining iron (Fe), and inevitable impurities, maintaining and extracting the slab, recrystallized-region-rolling the maintained and extracted slab in a temperature range of Tnr or higher, non-recrystallized-region-rolling the recrystallized-region-rolled material at a total reduction ratio of 30% or more, and cooling the non-recrystallized-region-rolled steel plate to a temperature range of (Bs - 80°C) to Bs.

### Slab Reheating, Maintaining and Extracting

The slab according to the present invention has the same alloy composition as the alloy composition of the steel plate described above, and a description of the alloy composition of the slab according to the present invention is thus replaced by the description of the alloy composition of the steel plate described above.

Since the slab reheating is a process of heating a steel in order to smoothly perform the subsequent rolling processes and secure desired physical properties of the steel plate, a heating process needs to be performed within an appropriate temperature range according to a purpose. A lower limit of a slab reheating temperature needs to be determined in consideration of whether or not it is a temperature at which precipitated elements may be sufficiently dissolved in the steel. In particular, since the slab according to the present invention essentially contains niobium (Nb) in order to secure high strength properties, the lower limit of the slab reheating temperature is limited to 1140°C in consideration of a resoluble temperature of niobium (Nb). On the other hand, when the slab reheating temperature is excessively high, the austenite grains become excessively coarse, which may cause a problem that grains of a final steel plate are excessively increased. Thus, in the present invention, an upper limit of the slab reheating temperature is limited to 1200°C.

The reheated slab is subjected to a maintaining and extracting process, if necessary, and a maintaining and extracting temperature of the slab is limited to a temperature range of 1140 to 1200°C for reasons similar to those of the slab reheating temperature.

### Recrystallized-Region-Rolling

The recrystallized-region-rolling is performed in a temperature range of Tnr or more. In the present invention, Tnr refers to a lower limit of a temperature range at which recrystallization of austenite occurs. That is, the recrystallized-region-rolling is performed in a temperature range of an austenite recrystallized region. The recrystallized-region-rolling may be performed in multiple passes, and rolling may be performed at an average reduction ratio of 10% or more per pass. The reason is that when the average reduction ratio per pass is less than 10%, a grain size of recrystallized austenite becomes coarse, which may cause a decrease in toughness of the final steel plate.

The recrystallized-region-rolled material may be cooled to a temperature range of Tnr or lower under a cooling condition of air cooling. That is, the recrystallized-region-rolled material is not immediately subjected to non-recrystallized-region-rolling, and may wait for a predetermined time to be cooled to a temperature range of a non-recrystallized region by air cooling. The reason is that when a rolling force is applied in the corresponding section, partial recrystallization may occur, such that a brittle fracture due to a coarse austenite grain size may occur.

### Non-recrystallized-Region-Rolling

The non-recrystallized-region-rolling is performed on the recrystallized-region-rolled material. A start temperature of the non-recrystallized-region-rolling is Tnr or lower, and an end temperature of the non-recrystallized-region-rolling is (Ar3+100°C). The non-recrystallized-region-rolling is a process for elongating austenite produced by recrystallized-region-rolling to be elongate and forming a deformed structure in a grain to obtain fine ferrite and bainite, and strength, an elongation ratio and brittle fracture arrestability of the steel plate may be effectively improved by the non-recrystallized-region-rolling.

The lower the end temperature of the non-recrystallized-zone-rolling, the higher the degree of deformation of the austenite, which is effective in improving low-temperature fracture toughness, but when the end temperature of the non-recrystallized-zone-rolling is excessively low, low-strength ferrite is produced, which is disadvantageous in securing strength. Thus, in the present invention, the end temperature of the non-recrystallized-zone-rolling may be limited to (Ar3 + 50°C) or higher.

In addition, a rolling reduction of the non-recrystallized-region-rolling is an important factor in securing low-temperature toughness of the steel. In the present invention, the rolling reduction of the non-recrystallized-region-rolling is limited to 30% or more in order to secure low-temperature DWTT percent ductile fracture characteristics according to refinement of grain sizes of a final steel. Since it is effective in improving low-temperature toughness that the rolling reduction of the non-recrystallized-region-rolling becomes larger, an upper limit of the rolling reduction of the non-recrystallized-region-rolling may not be limited. However, when the rolling reduction of the non-recrystallized-region-rolling exceeds a predetermined level, an effect of the refinement of the grain size is saturated, but a rolling reduction of the recrystallized-region-rolling is relatively decreased. Thus, in the present invention, the rolling reduction in the non-recrystallized-region-rolling may be limited to 90% or less.

### Cooling

The non-recrystallized-region-rolled steel plate is cooled from a cooling start temperature of (Ar3 + 30°C) or higher to a cooling stop temperature of (Bs - 80°C) to Bs. When the cooling start temperature is excessively low, a large amount of ferrite having low strength is produced, and accordingly, strength of the steel plate may be significantly decreased. Thus, in the present invention, the cooling starts in a temperature range of (Ar3 + 30°C) or higher.

In addition, since the steel plate according to the present invention has a final thickness less than 20 mm, it is most preferable in terms of strength and an elongation ratio to stop cooling in a temperature range of (Bs - 80°C) to Bs. The reason is that when the cooling stop temperature is lower than (Bs - 80°C), acicular ferrite and bainite having a high angle grain boundary formed to be coarse and a low angle grain boundary are formed in a large amount, such that an elongation ratio may be decreased, and when the cooling stop temperature exceeds Bs, an amount of bainite produced is small, such that strength of the steel plate may not be secured. The steel plate may be quenched to the cooling stop temperature of (Bs - 80°C) to Bs, then cooled to room temperature by air cooling or radiation cooling.

In addition, the cooling of the present invention is performed at a cooling rate of 10 to 50°C/s. The reason is that when the cooling rate is less than 10°C/s, a fraction of equiaxed ferrite is significantly increased, such that high strength characteristics of the steel plate may not be effectively secured. In terms of a facility condition and economy, an upper limit of the cooling rate is limited to 50°C/s.

The steel plate manufactured by the manufacturing method described above may contain ferrite and bainite as a microstructure, and further contain martensite-austenite constituent. Fractions of the ferrite and the bainite is 20 to 60 area% and 35 to 75 area%, respectively, and a fraction of the martensite-austenite constituent is 5 area% or less. In addition, the steel plate manufactured by the manufacturing method described above has a grain size of 70 um or less in upper 80% of high angle grain sizes based on 15° in a central portion of the steel plate.

Therefore, the steel plate manufactured by the manufacturing method described above has a thickness less than 20 mm, and has a yield strength of 485 MPa or more, a total elongation ratio of 28% or more, and a uniform elongation ratio of 9% or more with respect to a rolling orthogonal direction, and has a DWTT percent ductile fracture of 85% or more at -30°C with respect to the rolling orthogonal direction of the steel plate. Therefore, according to the manufacturing method according to an exemplary embodiment in the present invention, a steel plate particularly suitable as a material for a pipeline by effectively securing strength, low-temperature fracture toughness, and an elongation ratio in spite of having the thickness less than 20 mm is provided.

### [Mode for Invention]

Hereinafter, the present invention will be described in more detail through Inventive Example. However, it is to be noted that Inventive Example to be described later is for illustrating and embodying the present invention and is not intended to limit the scope of the present invention.

### (Inventive Example)

Slabs having alloy compositions of Table 1 and having a thickness of 250 mm were manufactured, and steel plate specimens having thicknesses of 11 mm, 11.5 mm, and 22 mm, respectively, were manufactured by applying process conditions of Table 3. In this case, the slabs were manufactured by applying process conditions used for manufacturing a general slab, and recrystallized-region-rolling was performed by applying a condition of an average rolling reduction per pass of 10% or more in a temperature range of Tnr or higher for all specimens. In addition, air cooling to a non-recrystallized region temperature range after the recrystallized-region-rolling was applied to all specimens. An Tnr temperature, an Ar3 temperature, and a Bs temperature were calculated on the basis of each alloy composition in Table 1 and shown in Table 2, and Equations used for calculating the Tnr temperature, the Ar3 temperature, and the Bs temperature of Table 2 were separately described below Table 2.

**[Table 1]**

| Ste el Typ e | Alloy Composition (wt%) | | | | | | | | | | | | | Div isi on |
|---|---|---|---|---|---|---|---|---|---|---|---|---|---|---|
| | C | Si | Mn | P | S | Ni | Cr | Mo | Nb | Al | Ca | Ti | N | |
| A | 0.070 | 0.27 | 1.57 | 0.01 | 0.0020 | 0.10 | 0.10 | - | 0.049 | 0.023 | 0.0010 | 0.011 | 0.0032 | Inv ent ive Ste el |
| B | 0.074 | 0.25 | 1.66 | 0.013 | 0.0020 | 0.10 | 0.10 | - | 0.055 | 0.034 | 0.0011 | 0.014 | 0.0044 | |
| C | 0.050 | 0.25 | 1.58 | 0.012 | 0.0019 | 0.10 | 0.11 | 0.08 | 0.048 | 0.023 | 0.0010 | 0.013 | 0.0043 | |
| D | 0.060 | 0.24 | 1.55 | 0.011 | 0.0019 | 0.10 | 0.10 | 0.08 | 0.041 | 0.026 | 0.0013 | 0.014 | 0.0041 | |
| E | 0.050 | 0.25 | 1.52 | 0.012 | 0.0018 | 0.10 | 0.10 | 0.08 | 0.041 | 0.024 | 0.0010 | 0.014 | 0.0044 | |
| F | 0.09 | 0.34 | 1.45 | 0.010 | 0.0011 | 0.17 | 0.1 | - | 0.045 | 0.027 | 0.0010 | 0.016 | 0.0041 | |
| G | 0.050 | 0.26 | 1.57 | 0.010 | 0.0020 | 0.10 | 0.11 | 0.08 | 0.028 | 0.028 | 0.0010 | 0.012 | 0.0046 | Com par ati ve Ste el |
| H | 0.040 | 0.26 | 1.24 | 0.008 | 0.0010 | 0.14 | 0.2 | 0.07 | 0.04 | 0.030 | 0.0007 | 0.012 | 0.0046 | |
| I | 0.060 | 0.25 | 2.10 | 0.0075 | 0.0015 | 0.3 | 0.15 | 0.10 | 0.050 | 0.030 | 0.0016 | 0.015 | 0.0050 | |

**[Table 2]**

| Steel Type | Tnr (°C) | Ar3 (°C) | Ar3 + 30 (°C) | Ar3 + 100 (°C) | Bs (°C) | Bs - 80 (°C) |
|---|---|---|---|---|---|---|
| A | 1014 | 767 | 797 | 867 | 659 | 579 |
| B | 1060 | 760 | 790 | 860 | 650 | 570 |
| C | 1009 | 771 | 801 | 871 | 656 | 576 |
| D | 985 | 771 | 801 | 871 | 657 | 577 |
| E | 976 | 776 | 806 | 876 | 662 | 582 |
| F | 985 | 767 | 797 | 867 | 662 | 582 |
| G | 911 | 772 | 802 | 872 | 657 | 577 |
| H | 963 | 796 | 826 | 896 | 683 | 603 |
| I | 1028 | 718 | 748 | 818 | 595 | 515 |

$\begin{matrix}Tnr \left(°C\right) = 887 + 464 * \left[C\right] + 6445 * \left[Nb\right] \\ - 644 * {\left[Nb\right]}^{\left(1/2\right)} + 732 * \left[V\right] - 230 * {\left[V\right]}^{\left(1/2\right)} + 890 * \left[Ti\right] + 363 * \left[Al\right] \\ - 357 * \left[Si\right]\end{matrix}$ $\begin{matrix}Ar3 \left(°C\right) = 910 - 273 * \left[C\right] - 74 * \left[Mn\right] - \\ 57 * \left[Ni\right] - 16 * \left[Cr\right] - 9 * \left[Mo\right] - 5 \left[Cu\right]\end{matrix}$ $\begin{matrix}Bs \left(°C\right) = 830 - 270 * \left[C\right] - 90 * \left[Mn\right] - \\ 37 * \left[Ni\right] - 70 * \left[Cr\right] - 83 * \left[Mo\right]\end{matrix}$

(In Equations 1 to 3, [C], [Si], [Mn], [Al], [Ti], [Nb], [V], [Cr], [Mo], and [Cu] refer to wt% of respective alloy compositions, and when a corresponding alloy composition is not contained, calculation is performed by replacing a value of the corresponding alloy composition with 0.)

**[Table 3]**

| Spe cim en | Steel Type | Thickness (mm) of Steel Plate | Slab Heating Tempera ture (°C) | Start Temperature (°C) of Non-recrystalli zed-Region-Rolling | Cumulative Rolling Reduction (%) of Non-recrystalliz ed-Region-Rolling | End Temperature (°C) of Non-recrystalli zed-Region-Rolling | Cooli ng Start Tempe ratur e (°C) | Cooli ng Stop Tempe ratur e (°C) | Cooling Rate (°C/s) | Remar k |
|---|---|---|---|---|---|---|---|---|---|---|
| 1 | A | 11.5 | 1150 | 1000 | 42.5 | 915 | 810 | 590 | 36 | Inven tive Examp le |
| 2 | A | 11.5 | 1170 | 1000 | 42.5 | 915 | 820 | 640 | 36 | |
| 3 | A | 11.5 | 1160 | 1000 | 50 | 875 | 800 | 580 | 43 | |
| 4 | B | 11.5 | 1160 | 1035 | 56 | 915 | 805 | 615 | 32 | |
| 5 | B | 11.5 | 1165 | 1035 | 56 | 915 | 820 | 610 | 35 | |
| 6 | B | 11.5 | 1150 | 1025 | 56 | 875 | 800 | 625 | 35 | |
| 7 | C | 11 | 1160 | 990 | 39 | 925 | 830 | 580 | 30 | |
| 8 | C | 11 | 1150 | 995 | 39 | 920 | 825 | 635 | 30 | |
| 9 | D | 11 | 1160 | 985 | 31 | 920 | 830 | 620 | 30 | |
| 10 | E | 11 | 1150 | 975 | 31 | 920 | 825 | 590 | 30 | |
| 11 | E | 11 | 1160 | 975 | 31 | 920 | 830 | 620 | 30 | |
| 12 | F | 11 | 1150 | 981 | 39 | 875 | 805 | 620 | 35 | |
| 13 | C | 11 | 1160 | 1000 | 50 | 875 | 795 | 460 | 42 | Compa rativ e Examp le |
| 14 | D | 11 | 1150 | 975 | 31 | 920 | 825 | 550 | 30 | |
| 15 | D | 11 | 1150 | 970 | 31 | 920 | 825 | 510 | 30 | |
| 16 | D | 11 | 1160 | 983 | 50 | 863 | 771 | 685 | 30 | |
| 17 | E | 11 | 1150 | 975 | 31 | 920 | 820 | 530 | 30 | |
| 18 | G | 11 | 1170 | 910 | 12 | 910 | 830 | 470 | 30 | |
| 19 | G | 11 | 1150 | 910 | 12 | 910 | 830 | 580 | 30 | |
| 20 | H | 11 | 1159 | 954 | 0 | 954 | 819 | 491 | 47 | |
| 21 | I | 11 | 1160 | 1020 | 45 | 920 | 830 | 570 | 30 | |
| 22 | A | 22 | 1150 | 945 | 98 | 835 | 775 | 610 | 23 | |
| 23 | D | 22 | 1144 | 935 | 78 | 827 | 767 | 617 | 21 | |

For each specimen of Table 3, a microstructure, a yield strength and a tensile strength, an elongation ratio, and a DWTT percent shear at -30°C were measured and shown in Table 4. The microstructure of each specimen was evaluated using an optical microscope structure photograph and an electron backscatter diffraction (EBSD) grain size distribution chart. The yield strength, the tensile strength, and the elongation ratio were evaluated by performing a room temperature tensile test on each specimen. A yield strength and a tensile strength shown in Table 4 refer to measured values with respect to a rolling orthogonal direction, respectively. In addition, tensile properties and a percent ductile fracture were evaluated by performing a DWTT test at -30°C on each specimen.

**[Table 4]**

| Spe cim en | Ste el Typ e | Ferrite (area%) | Bainite (area%) | M/A (area%) | Grain Size (µm) of Upper 80% of High Angle Grains | Yield Strengt h (MPa) | Tensile Strengt h (MPa) | Yield Ratio (%) | Elong ation Ratio (%) | Unifor m Elonga tion Ratio (%) | DWTT (%) at -30°C | Rem ark |
|---|---|---|---|---|---|---|---|---|---|---|---|---|
| 1 | A | 25 | 71.0 | 4.0 | 52.0 | 524 | 667 | 79 | 33 | 9.0 | 100 | Inv ent ive Exa mpl e |
| 2 | A | 42 | 54.5 | 3.5 | 40.5 | 508 | 635 | 80 | 36 | 10.5 | 100 | |
| 3 | A | 28 | 67.5 | 4.5 | 46.5 | 541 | 671 | 81 | 35 | 9.6 | 100 | |
| 4 | B | 32 | 63.6 | 4.4 | 62.1 | 525 | 671 | 78 | 33 | 9.0 | 100 | |
| 5 | B | 43 | 52.8 | 4.2 | 57.9 | 529 | 667 | 79 | 34 | 9.5 | 100 | |
| 6 | B | 52 | 43.5 | 4.5 | 56.6 | 528 | 653 | 81 | 36 | 9.9 | 99 | |
| 7 | C | 23 | 72.8 | 4.2 | 67.1 | 487 | 643 | 76 | 33 | 9.2 | 98 | |
| 8 | C | 30 | 65.7 | 4.3 | 48.5 | 489 | 620 | 79 | 34 | 9.7 | 99 | |
| 9 | D | 23 | 72.7 | 4.3 | 60.1 | 505 | 638 | 79 | 33 | 9.1 | 100 | |
| 10 | E | 24 | 71.5 | 4.5 | 48.5 | 485 | 614 | 79 | 31 | 9.7 | 100 | |
| 11 | E | 28 | 67.7 | 4.3 | 42.0 | 495 | 613 | 81 | 36 | 10.9 | 100 | |
| 12 | F | 31 | 64.8 | 4.2 | 45.1 | 536 | 625 | 86 | 36 | 10.5 | 95 | |
| 13 | C | 17 | 78.3 | 4.7 | 86.1 | 620 | 730 | 85 | 28 | 7.7 | 100 | Com par ati ve Exa mpl e |
| 14 | D | 15 | 80.5 | 4.5 | 89.5 | 501 | 651 | 77 | 28 | 7.6 | 100 | |
| 15 | D | 18 | 77.7 | 4.3 | 75.2 | 500 | 628 | 80 | 32 | 8.3 | 100 | |
| 16 | D | 75 | 22.9 | 2.1 | 90.5 | 455 | 570 | 80 | 42 | 13.0 | 92 | |
| 17 | E | 22 | 74.0 | 4.0 | 76.5 | 492 | 632 | 78 | 28 | 8.2 | 100 | |
| 18 | G | 24 | 72 | 4.0 | 93 | 524 | 656 | 80 | 28 | 6.3 | 75 | |
| 19 | G | 26 | 69.8 | 4.2 | 82.5 | 502 | 620 | 81 | 32 | 7.9 | 80 | |
| 20 | H | 28 | 67.9 | 4.1 | 78.0 | 528 | 606 | 87 | 30 | 8.0 | 50 | |
| 21 | I | 12 | 81.8 | 6.2 | 89.1 | 624 | 796 | 78 | 28 | 6.8 | 91 | |
| 22 | A | 65 | 31.2 | 3.8 | 58.6 | 475 | 568 | 84 | 47 | 13.0 | 100 | |
| 23 | D | 66 | 30.5 | 3.5 | 65.1 | 470 | 565 | 83 | 48 | 13.5 | 100 | |

It may be confirmed that Specimens 1 to 12 satisfying the alloy composition and process conditions of the present invention contain 20 to 60 area% of ferrite and 35 to 75 area% of bainite as a microstructure, contain 5 area% or less of island martensite, and have a grain size of 70 µm or less in upper 80% of high angle grain sizes based on 15° in a central portion of a steel plate, a yield strength of 485MPa or more, a total elongation ratio of 28% or more, a uniform elongation ratio of 9% or more with respect to a rolling orthogonal direction, and a DWTT percent shear of 85% or more at -30°C with respect to the rolling orthogonal direction, and thus, has physical properties particularly suitable as a material for a pipeline provided in a cryogenic environment.

Specimens 13 to 15 and 17 are specimens in a case where the alloy composition of the present invention is satisfied, but cooling is performed in a temperature range lower than the cooling start temperature or the cooling end temperature of the present invention. It may be confirmed that in a case of Specimens 13 to 15 and 17, ferrite less than 20 area% and bainite more than 75 area% were formed, a grain size of upper 80% of high angle grain sizes based on 15° in a central portion of a steel plate exceeded 70 um, and a uniform elongation ratio was thus less than 9%.

Specimen 16 is a specimen in a case where the alloy composition of the present invention is satisfied, but non-recrystallized-region-rolling was performed in a temperature range lower than the end temperature of the non-recrystallized-region-rolling of the present invention, and cooling started in a temperature range lower than the cooling start temperature of the present invention, such that cooling ended in a temperature range higher than the cooling stop temperature of the present invention. It may be confirmed that in a case of Specimen 16, ferrite more than 60 area% was formed, such that a yield strength was less than 485 MPa.

It may be confirmed that Specimens 18 to 21, which are specimens that do not satisfy the alloy composition and the process condition of the present invention, do not secure a microstructure and physical properties desired by the present invention.

It may be confirmed that Specimens 22 and 23 satisfy the alloy composition of the present invention, but have a thickness of a steel plate exceeding 20 mm, such that ferrite is excessively formed.

FIG. 1 is a photograph of Specimen 2 observed with an optical microscope, while FIG. 2 is graphs illustrating results obtained by measuring high angle grain boundary grain sizes based on 15° of Specimen 2 using an EBSD. As illustrated in the graphs of FIG. 2, it may be confirmed that an average grain size of high angle grain boundaries of Specimen 2 is 22.3 um and a grain size of upper 80% of the high angle grain boundaries is 40.5 µm.

FIG. 3 is a photograph of Specimen 18 observed with an optical microscope, and FIG. 4 is graphs illustrating results obtained by measuring high angle grain boundary grain sizes based on 15° of Specimen 18 using an EBSD. As illustrated in the graphs of FIG. 4, it may be confirmed that an average grain size of high angle grain boundaries of Specimen 18 is 38 um and a grain size of upper 80% of the high angle grain boundaries is 93 um.

Therefore, according to an exemplary embodiment in the present invention, the steel plate particularly suitable as the material for a pipeline by having the yield strength of 485MPa or more, the total elongation ratio of 28% or more, the uniform elongation ratio of 9% or more with respect to the rolling orthogonal direction, and the DWTT percent ductile fracture of 85% or more at -30°C with respect to the rolling orthogonal direction of the steel plate in spite of having a thickness less than 20 mm, and the manufacturing method therefor may be provided.

While the present invention has been described in detail through exemplary embodiment, other types of exemplary embodiments are also possible. Therefore, the scope of the invention is only defined by the claims.

## Claims

1. A high-strength steel plate having excellent low-temperature fracture toughness and elongation ratio, comprising:
by wt%, 0.05 to 0.1% of carbon (C), 0.05 to 0.5% of silicon (Si), 1.4 to 2.0% of manganese (Mn), 0.01 to 0.05% of aluminum (Al), 0.005 to 0.02% of titanium (Ti), 0.002 to 0.01% of nitrogen (N), 0.04 to 0.07% of niobium (Nb), 0.05 to 0.3% of chromium (Cr), 0.05 to 0.4% of nickel (Ni), 0.02% or less of phosphorus (P), 0.005% or less of sulfur (S), 0.0005 to 0.004% of calcium (Ca), remaining iron (Fe), and inevitable impurities; and
20 to 60 area% of ferrite, 35 to 75 area% of bainite and 5 area% or less of martensite-austenite constituent as a microstructure,
wherein a grain size of upper 80% of high angle grain sizes based on 15° in a central portion of the high-strength steel plate is 70 µm or less,
wherein the steel plate optionally further comprises 0.3 wt% or less of molybdenum (Mo),
wherein a thickness of the high-strength steel plate is less than 20 mm,
wherein a yield strength of the high-strength steel plate is 485 MPa or more,
wherein a total elongation ratio of the high-strength steel plate is 28% or more,
wherein a uniform elongation ratio of the high-strength steel plate with respect to a rolling orthogonal direction is 9% or more, and
wherein a drop weight tearing test (DWTT) percent ductile shear of the high-strength steel plate at -30°C with respect to a rolling orthogonal direction of the steel plate is 85% or more,
wherein the yield strength and the elongation ratio were evaluated by performing a room temperature tensile test with respect to a rolling orthogonal direction.

2. A manufacturing method for a high-strength steel plate having excellent low-temperature fracture toughness and elongation ratio of claim 1, comprising:
reheating a slab comprising, by wt%, 0.05 to 0.1% of carbon (C), 0.05 to 0.5% of silicon (Si), 1.4 to 2.0% of manganese (Mn), 0.01 to 0.05% of aluminum (Al), 0.005 to 0.02% of titanium (Ti), 0.002 to 0.01% of nitrogen (N), 0.04 to 0.07% of niobium (Nb), 0.05 to 0.3% of chromium (Cr), 0.05 to 0.4% of nickel (Ni), 0.02% or less of phosphorus (P), 0.005% or less of sulfur (S), 0.0005 to 0.004% of calcium (Ca), remaining iron (Fe), and inevitable impurities;
maintaining and extracting the slab;
recrystallized-region-rolling the maintained and extracted slab in a temperature range of Tnr or higher;
non-recrystallized-region-rolling the recrystallized-region-rolled material at a total reduction ratio of 30% or more; and
cooling the non-recrystallized-region-rolled steel plate to a temperature range of (Bs - 80°C) to Bs, wherein the non-recrystallized-region-roll starts in a temperature range of Tnr or lower and ends in a temperature range of (Ar3 + 100°C) or higher,
wherein the slab plate optionally further comprises 0.3 wt% or less of molybdenum (Mo),
wherein a reheating temperature range of the slab is 1140 to 1200°C,
wherein a maintaining and extracting temperature range of the slab is 1140 to 1200°C,
wherein the non-recrystallized-region-rolled steel plate is cooled at a cooling rate of 10 to 50°C/s,
wherein the cooling of the non-recrystallized-region-rolled steel plate starts in the temperature range of (Ar3 + 30°C) or higher, and
wherein the Tnr, Ar3 and Bs is calculated by Equations 1 to 3 below.Equation 1: Tnr (°C) = 887 + 464*[C] + 6445*[Nb] - 644*[Nb](^{1/2}) + 732*[V] - 230*[V]^{(1/2)} + 890*[Ti] + 363*[A1] - 357*[Si] $Ar3 \left(°C\right) = 910 - 273 ∗ \left[C\right] - 74 ∗ \left[Mn\right] - 57 ∗ \left[Ni\right] - 16 ∗ \left[Cr\right] - 9 ∗ \left[Mo\right] - 5 \left[Cu\right]$ $Bs \left(°C\right) = 830 - 270 ∗ \left[C\right] - 90 ∗ \left[Mn\right] - 37 ∗ \left[Ni\right] - 70 ∗ \left[Cr\right] - 83 ∗ \left[Mo\right]$
where, [C], [Si], [Mn], [Al], [Ti], [Nb], [V], [Cr], [Mo], and [Cu] refer to wt% of respective alloy compositions, and when a corresponding alloy composition is not contained, calculation is performed by replacing a value of the corresponding alloy composition with 0.

3. The manufacturing method of claim 2, wherein the recrystallized-region-rolling is performed in a accumulation of passes, and an average reduction ratio of each of the passes is 10% or more.

4. The manufacturing method of claim 2, wherein the recrystallized-region-rolled material is cooled to a temperature range of Tnr or lower by air cooling.

## Patentansprüche

1. Hochfestes Stahlblech mit ausgezeichneter Tieftemperatur-Bruchzähigkeit und ausgezeichnetem Dehnungsverhältnis, umfassend:
in Gew.-% 0,05 bis 0,1 % Kohlenstoff (C), 0,05 bis 0,5 % Silicium (Si), 1,4 bis 2,0 % Mangan (Mn), 0,01 bis 0,05 % Aluminium (Al), 0,005 bis 0,02 % Titan (Ti), 0,002 bis 0,01 % Stickstoff (N), 0,04 bis 0,07 % Niob (Nb), 0,05 bis 0,3 % Chrom (Cr), 0,05 bis 0,4 % Nickel (Ni), 0,02 % oder weniger Phosphor (P), 0,005 % oder weniger Schwefel (S), 0,0005 bis 0,004 % Calcium (Ca), restliches Eisen (Fe) und unvermeidliche Verunreinigungen; und
20 bis 60 Flächen-% Ferrit, 35 bis 75 Flächen-% Bainit und 5 Flächen-% oder weniger Martensit-Austenit-Komponente als Mikrogefüge,
wobei eine Korngröße der oberen 80 % der
Großwinkelkorngrößen auf der Basis von 15° in einem zentralen Abschnitt des hochfesten Stahlblechs 70 µm oder weniger beträgt,
wobei das Stahlblech optional ferner 0,3 Gew.-% oder weniger Molybdän (Mo) umfasst,
wobei eine Dicke des hochfesten Stahlblechs weniger als 20 mm beträgt,
wobei eine Streckgrenze des hochfesten Stahlblechs 485 MPa oder mehr beträgt,
wobei ein Gesamtdehnungsverhältnis des hochfesten Stahlblechs 28 % oder mehr beträgt,
wobei ein gleichmäßiges Dehnungsverhältnis des hochfesten Stahlblechs in Bezug auf eine Walz-Orthogonal-Richtung 9 % oder mehr beträgt, und
wobei eine prozentuale duktile Scherung beim Fallgewichts-Reißversuch (DWTT) des hochfesten Stahlblechs bei -30 °C in Bezug auf eine Walz-Orthogonal-Richtung des Stahlblechs 85 % oder mehr beträgt,
wobei die Streckgrenze und das Dehnungsverhältnis bewertet wurden, indem ein Raumtemperatur-Zugversuch in Bezug auf eine Walz-Orthogonal-Richtung durchgeführt wurde.

2. Verfahren zur Herstellung eines hochfesten Stahlblechs mit ausgezeichneter Tieftemperatur-Bruchzähigkeit und ausgezeichnetem Dehnungsverhältnis nach Anspruch 1, umfassend:
Wiedererwärmen einer Bramme, umfassend in Gew.-% 0,05 bis 0,1 % Kohlenstoff (C), 0,05 bis 0,5 % Silicium (Si), 1,4 bis 2,0 % Mangan (Mn), 0,01 bis 0,05 % Aluminium (Al), 0,005 bis 0,02 % Titan (Ti), 0,002 bis 0,01 % Stickstoff (N), 0,04 bis 0,07 % Niob (Nb), 0,05 bis 0,3 % Chrom (Cr), 0,05 bis 0,4 % Nickel (Ni), 0,02 % oder weniger Phosphor (P), 0,005 % oder weniger Schwefel (S), 0,0005 bis 0,004 % Calcium (Ca), restliches Eisen (Fe) und unvermeidliche Verunreinigungen;
Halten und Extrahieren der Bramme;
Walzen des rekristallisierten Bereichs der gehaltenen und extrahierten Bramme in einem Temperaturbereich von Tnr oder höher;
Walzen des nicht rekristallisierten Bereichs des im rekristallisierten Bereich gewalzten Materials mit einem Gesamtreduktionsverhältnis von 30 % oder mehr; und
Abkühlen des im nicht rekristallisierten Bereich gewalzten Stahlblechs auf einen Temperaturbereich von (Bs - 80 °C) bis Bs,
wobei das Walzen des nicht rekristallisierten Bereichs in einem Temperaturbereich von Tnr oder niedriger beginnt und in einem Temperaturbereich von (Ar3 + 100 °C) oder höher endet,
wobei das Brammenblech optional ferner 0,3 Gew.-% oder weniger Molybdän (Mo) umfasst,
wobei ein Wiedererwärmungs-Temperaturbereich der Bramme 1140 bis 1200 °C beträgt,
wobei ein Halte- und Extraktions-Temperaturbereich der Bramme 1140 bis 1200 °C beträgt,
wobei das im nicht rekristallisierten Bereich gewalzte Stahlblech mit einer Abkühlungsrate von 10 bis 50 °C/s abgekühlt wird,
wobei das Abkühlen des im nicht rekristallisierten Bereich gewalzten Stahlblechs im Temperaturbereich von (Ar3 + 30 °C) oder höher beginnt, und
wobei Tnr, Ar3 und Bs durch die nachstehenden Gleichungen 1 bis 3 berechnet werden: $\begin{matrix}Tnr \left(°C\right) = 887 + 464 * \left[C\right] + 6445 * \left[Nb\right] - \\ 644 * {\left[Nb\right]}^{\left(1/2\right)} + 732 * \left[V\right] - 230 * {\left[V\right]}^{\left(1/2\right)} + 890 * \left[Ti\right] + 363 * \left[Al\right] \\ - 357 * \left[Si\right]\end{matrix}$ $\begin{matrix}Ar 3 \left(°C\right) = 910 - 273 * \left[C\right] - 74 * \left[Mn\right] - 57 * \left[Ni\right] \\ - 16 * \left[Cr\right] - 9 * \left[Mo\right] - 5 \left[Cu\right]\end{matrix}$ $\begin{matrix}Bs \left(°C\right) = 830 - 270 * \left[C\right] - 90 * \left[Mn\right] - 37 * \left[Ni\right] - \\ 70 * \left[Cr\right] - 83 * \left[Mo\right]\end{matrix}$
wobei sich [C], [Si], [Mn], [Al], [Ti], [Nb], [V], [Cr], [Mo] und [Cu] auf Gew.-% der jeweiligen Legierungszusammensetzungen beziehen und wobei, wenn eine entsprechende Legierungszusammensetzung nicht enthalten ist, die Berechnung durchgeführt wird, indem ein Wert der entsprechenden Legierungszusammensetzung durch 0 ersetzt wird.

3. Herstellungsverfahren nach Anspruch 2, wobei das Walzen des rekristallisierten Bereichs in einer Ansammlung von Durchgängen durchgeführt wird und ein durchschnittliches Reduktionsverhältnis von jedem der Durchgänge 10 % oder mehr beträgt.

4. Herstellungsverfahren nach Anspruch 2, wobei das im rekristallisierten Bereich gewalzte Material durch Luftkühlen auf einen Temperaturbereich von Tnr oder niedriger abgekühlt wird.

## Revendications

1. Plaque d'acier à haute résistance présentant une excellente ténacité à la rupture à basse température et un excellent rapport d'allongement, comprenant :
en % en poids, 0,05 à 0,1 % de carbone (C), 0,05 à 0,5 % de silicium (Si), 1,4 à 2,0 % de manganèse (Mn), 0,01 à 0,05 % d'aluminium (Al), 0,005 à 0,02 % de titane (Ti), 0,002 à 0,01 % d'azote (N), 0,04 à 0,07 % de niobium (Nb), 0,05 à 0,3 % de chrome (Cr), 0,05 à 0,4 % de nickel (Ni), 0,02 % ou moins de phosphore (P), 0,005 % ou moins de soufre (S), 0,0005 à 0,004 % de calcium (Ca), un reste de fer (Fe), et des impuretés inévitables ; et
20 à 60 % en aire de ferrite, 35 à 75 % en aire de bainite et 5 % en aire ou moins de constituant martensite-austénite en tant que microstructure,
dans laquelle une taille de grain de 80 % supérieure des tailles de grain à angle élevé sur la base de 15° dans une portion centrale de la plaque d'acier à haute résistance est de 70 µm ou moins,
la plaque d'acier comprenant en outre facultativement 0,3 % en poids ou moins de molybdène (Mo),
dans laquelle une épaisseur de la plaque d'acier à haute résistance est inférieure à 20 mm,
dans laquelle une limite d'élasticité de la plaque d'acier à haute résistance est de 485 MPa ou plus,
dans laquelle un rapport d'allongement total de la plaque d'acier à haute résistance est de 28 % ou plus,
dans laquelle un rapport d'allongement uniforme de la plaque d'acier à haute résistance par rapport à une direction orthogonale de laminage est de 9 % ou plus, et
dans laquelle un pourcentage de cisaillement ductile par essai de rupture par chute de poids (DWTT) de la plaque d'acier à haute résistance à -30 °C par rapport à la direction orthogonale de laminage de la plaque d'acier est de 85 % ou plus,
dans laquelle la limite d'élasticité et le rapport d'allongement ont été évalués en réalisant un essai de traction à température ambiante par rapport à une direction orthogonale de laminage.

2. Procédé de fabrication d'une plaque d'acier à haute résistance présentant une excellente ténacité à la rupture à basse température et un excellent rapport d'allongement selon la revendication 1, comprenant :
le réchauffage d'une brame comprenant, en % en poids, 0,05 à 0,1 % de carbone (C), 0,05 à 0,5 % de silicium (Si), 1,4 à 2,0 % de manganèse (Mn), 0,01 à 0,05 % d'aluminium (Al), 0,005 à 0,02 % de titane (Ti), 0,002 à 0,01 % d'azote (N), 0,04 à 0,07 % de niobium (Nb), 0,05 à 0,3 % de chrome (Cr), 0,05 à 0,4 % de nickel (Ni), 0,02 % ou moins de phosphore (P), 0,005 % ou moins de soufre (S), 0,0005 à 0,004 % de calcium (Ca), un reste du fer (Fe), et des impuretés inévitables ;
le maintien et l'extraction de la brame ;
le laminage de région recristallisée de la plaque maintenue et extraite dans une plage de température de Tnr ou supérieure ;
le laminage de région non recristallisée du matériau ayant subi un laminage de région recristallisée à un rapport de réduction total de 30 % ou plus ; et
le refroidissement de la plaque d'acier ayant subi un laminage de région non recristallisée jusqu'à une plage de températures de (Bs - 80 °C) à Bs,
dans lequel le laminage de région non recristallisée commence dans une plage de température de Tnr ou inférieure et se termine dans une plage de température de (Ar3 +100 °C) ou supérieure,
dans lequel la plaque de brame comprend en outre facultativement 0,3 % en poids ou moins de molybdène (Mo),
dans lequel une plage de température de réchauffage de la brame est de 1140 à 1200 °C,
dans lequel une plage de température de maintien et d'extraction de la brame est de 1140 à 1200 °C,
dans lequel la plaque d'acier ayant subi un laminage de région non recristallisée est refroidie à une vitesse de refroidissement de 10 à 50 °C/s,
dans lequel le refroidissement de la plaque d'acier ayant subi un laminage de région non recristallisée commence dans la plage de température de (Ar3 + 30 °C) ou supérieure, et
dans lequel Tnr, Ar3 et Bs sont calculées par les équations 1 à 3 ci-dessous. $\begin{matrix}Tnr \left(°C\right) = 887 + 464 * \left[C\right] + \\ 6445 * \left[Nb\right] - 644 * {\left[Nb\right]}^{\left(1/2\right)} + 732 * \left[V\right] - 230 * {\left[V\right]}^{\left(1/2\right)} + 890 * \left[Ti\right] \\ + 363 * \left[Al\right] - 357 * \left[Si\right]\end{matrix}$ $\begin{matrix}Ar 3 \left(°C\right) = 910 - 273 * \left[C\right] - 74 * \left[Mn\right] - \\ 57 * \left[Ni\right] - 16 * \left[Cr\right] - 9 * \left[Mo\right] - 5 \left[Cu\right]\end{matrix}$ $\begin{matrix}Bs \left(°C\right) = 830 - 270 * \left[C\right] - 90 * \left[Mn\right] - \\ 37 * \left[Ni\right] - 70 * \left[Cr\right] - 83 * \left[Mo\right]\end{matrix}$
où [C], [Si], [Mn], [Al], [Ti], [Nb], [V], [Cr], [Mo] et [Cu] se réfèrent aux % en poids des compositions d'alliage respectives, et lorsqu'une composition d'alliage correspondante n'est pas contenue, le calcul est réalisé en remplaçant une valeur de la composition d'alliage correspondante par 0.

3. Procédé de fabrication selon la revendication 2, dans lequel le laminage de région recristallisée est réalisé en une accumulation de passes, et un rapport de réduction moyen de chacune des passes est de 10 % ou plus.

4. Procédé de fabrication selon la revendication 2, dans lequel le matériau ayant subi un laminage de région recristallisée est refroidi jusqu'à une plage de température de Tnr ou inférieure par refroidissement à l'air.
